

## 1

3,055,772

## TEXTILE YARN SIZING PROCESS

Simpey Kuramoto, St. Louis Park, Minn., assignor to  
General Mills, Inc., a corporation of Delaware  
No Drawing. Filed Dec. 1, 1960, Ser. No. 72,863  
6 Claims. (Cl. 117—139.5)

This invention relates to a novel textile sizing process.

In the weaving of yarns into fabrics, most yarns lack the strength and abrasion resistance necessary to weave efficiently under typical weaving conditions. To overcome these deficiencies, yarns are impregnated with a material called "size." Generally, the size is removed at the end of the weaving operation to yield a size-free fabric. Thus, it is important that the size lend the necessary strength and abrasion resistance and be readily removable from the fabric. Since end breaks are inevitable, ends that do break should be free of "fuzz balls" so that further weaving is not suspended in any way.

It is an object of this invention to provide a novel process for sizing textile yarns. It is another object of this invention to provide a sizing process wherein the size is easily removed. It is a further object of this invention to provide a yarn which is abrasion resistant and which weaves efficiently. Other objects will appear hereinafter.

The objects of this invention are accomplished by the process which comprises impregnating a textile yarn with cyanoethylated gluten and recovering a strong, abrasion resistant yarn obtained thereby. In accordance with the present invention, it was discovered that cyanoethylated gluten provides an excellent sizing compound for yarns.

As used herein, the term "cyanoethylated gluten" refers to the reaction product under aqueous alkaline conditions of gluten and acrylonitrile. This product may be prepared by reacting an aqueous alkaline gluten solution with acrylonitrile at room temperature. Details of such a preparation are described in U.S. 2,562,534, granted to John Robert Coffman on July 31, 1951.

Virtually any yarn may be sized by this process. Since excellent results are normally obtained with extremely inexpensive sizing agents in the case of natural fibers, the present invention is most useful in the sizing of synthetic fibers. Synthetic fibers generally are much more difficult to size than natural fibers due to the generally inert chemical composition and smooth physical structure of synthetic fibers. Typical synthetic fibers which are suitable for use in the present invention include cellulose acetate fibers, polyester fibers and polyamide fibers.

The sizing composition of the present invention may be applied to the yarn in a variety of ways. Generally, these methods are very well known in the art. A preferred method consists of passing a yarn through a solution of the size, subjecting the yarn to pressure to squeeze out the excess size and subsequently drying to remove the size solvent. The process of applying size is referred to as "slashing," by those in the art.

The size of the present invention is easily removed by washing in a detergent. Other methods of removing the size such as by enzymatic action may be employed if desired. In some instances, it is not desirable to remove the size, and here, the present size may be left on the yarn with no particular disadvantage.

The amount of size employed is not critical. Some improvement in weaving qualities is obtained even when extremely low concentrations of the sizing agent are employed. Generally, it is uneconomical and unnecessary to employ extremely large amounts of size. Normally, 4 to 8% by weight of the size, based on the weight of the yarn, is preferred. The amount of size employed is conveniently controlled by controlling the concentration of

## 2

size in the sizing solution and by removing excess solution by means of squeeze rolls. The use of squeeze rolls is preferred in any event in order to obtain more uniform impregnation of the yarn.

5 The size is most conveniently applied as an aqueous solution. It will be understood that the "solution" is actually a colloidal dispersion although generally referred to as solutions by those in the art. Preferably the solution contains 5 to 15% by weight of the cyanoethylated gluten. Other solvents may also be employed to dissolve the sizing agents if desired. The size may be applied to the yarn initially but is more conveniently applied after the yarn has been made into a warp.

Generally, better results are obtained when a small 15 amount of plasticizer is added to the yarn along with the sizing agents. The plasticizer yields a more flexible coating of the sizing agent. The plasticizer employed is not critical. Preferred plasticizers are the glycols such as ethylene glycol, glycerin propylene glycol, and esters 20 such as butyl adipate.

Sizing is best carried out at temperature somewhat 25 above room temperature. The preferred conditions are from 100 to 140° F. Higher temperature may be employed, but to no substantial advantage.

After slashing, the wet yarn is dried. This may be done by passing the treated yarn through a heated oven. A preferred method is to pass the yarn over a series of heated rolls or "cans" as they are referred to in the art. A series of these cans are placed substantially side by side and the yarn passed over one can and under the next etc.

The following examples are included to illustrate 35 various features of the present invention and the preferred embodiments thereof.

*Example I*

A 210 end warp having 143 ends per inch was prepared from 75 denier cellulose acetate yarn having 20 filaments per end and 5 twists per inch with a Z twist. 40 The warp was passed through an aqueous solution at 110° F., containing 9% by weight, based on the total composition, of cyanoethylated gluten and 1% by weight, based on the total composition of glycerin. The warp was passed through squeeze rolls and dried by passing over, under, etc., four rollers heated to 160° F., 180° F., 180° F., and 160° F., respectively. The sized warp which retained 8.5% by weight, of the size, was woven on a Draper XD loom operating at 172 picks per inch using the above cellulose acetate as fill. Fifty yards of fabric 45 were woven. There were 0.5 stop per ten yards on warp and no stops on the weaving. There were no thread breaks on the slashing step and 2 breaks on the weaving due to broken filaments. The picks per inch were 102% of the calculated concentration. The weaving efficiency 50 was calculated as 85%.

*Example II*

A 5600 end warp having 136 ends per inch was prepared from 75 denier cellulose acetate yarn having 20 filaments per end and 5 twists per inch with a Z twist. 60 The warp was slashed as in Example I with an aqueous sizing solution at 140° F. containing 6.48% by weight, based on the total composition, of cyanoethylated gluten and 0.72% by weight, based on the total composition, of glycerin. After passing through Quetsch rolls which exerted 1200 p.s.i. pressure on the warp, the slashed warp was dried and fed to a Draper XD loom operating at a fill density of 172 picks per inch using the above cellulose acetate as fill. The warp retained 5.4% by weight, of the size. The material shed from the weaving operation was 65 collected and found to be 4.5 grains per 10 yards. Dur- 70

ing the weaving of fifty yards of the fabric there were 2.2 loom stops per ten yards for the warp and no stop on the filling. In the 50 yards there were breaks on the slashing operation and 11 breaks on the weaving due to broken filaments. The weaving efficiency was calculated as 93.8%.

The foregoing examples are not to be interpreted as limitations on the scope of the present invention. Numerous variations will be apparent to those skilled in the art.

The process of the present invention is useful in producing sized yarn having improved weaving qualities.

The embodiments of the invention in which an exclusive property or privilege is claimed are defined as follows:

1. The process which comprises impregnating a textile 15  
yarn with cyanoethylated gluten, drying the yarn, and recovering a strong, abrasion resistant, sized yarn obtained thereby.

2. The process of claim 1 wherein the yarn is simultaneously impregnated with a plasticizer.

3. The process of claim 1 wherein the yarn is a cellulose acetate yarn.

4. The process of claim 1 wherein the textile yarn is polyester filament.

5. The process of sizing synthetic textile yarn which comprises passing said yarn through an aqueous solution of glycerin and cyanoethylated gluten, removing said 10  
yarn from said solution, drying the yarn, and recovering a strong, abrasion resistant, sized yarn obtained thereby.

6. A sizing composition consisting essentially of an aqueous solution of cyanoethylated gluten and a plasticizing amount of glycerin.

**References Cited in the file of this patent**

**UNITED STATES PATENTS**

2,562,534 Coffman ----- July 31, 1951